# EUROPEAN PATENT SPECIFICATION

(11) **EP 1 246 890 B1**
(45) Date of publication and mention of the grant of the patent: **23.08.2006**
(21) Application number: 00977195.7
(22) Date of filing: 13.11.2000
(51) Int. Cl.: C10G 45/04

(54) **PRESULFIDING HYDROPROCESSING CATALYST REPLACEMENT BATCHES**
VORSULFIDIERUNG VON WASSERSTOFFBEHANDLUNGS-KATALYSATORCHARGEN
CUVEES DE REMPLACEMENT D'HYDROTRAITEMENT DE PRESULFURATION D'UN CATALYSEUR

(30) Priority: 16.12.1999 US 465122
(43) Date of publication of application: 09.10.2002
(62) Divisional of application: 05027183.2
(73) Proprietor: Chevron U.S.A. Inc., San Ramon, CA 94583-2324 (US)
(72) Inventor: LEUNG, Pak, C., Lafayette, CA 94549 (US); EARLS, David, E., Pinole, CA 94564 (US); REYNOLDS, Bruce, Martinez, CA 94553 (US); JOHNSON, David, R., Petaluma, CA 94954 (US); BACHTEL, Robert, El Cerrito, CA 94530 (US); TRIMBLE, Harold, J., Panama City, FL 32411 (US)
(74) Representative: Nash, David Allan
(86) International application number: PCT/US2000/031131
(87) International publication number: WO 2001/044408

(56) References cited:
- EP-A- 0 785 022
- WO-A-93/03117
- US-A- 3 873 441

## Description

### Background of the Invention

The present invention relates to a method for extending the catalytic life of catalyst used in hydroprocessing of a hydrocarbon feed stream. More particularly, the present invention provides for a method for presulfiding hydroprocessing catalyst in order to improve operability, reduce catalyst fouling rate, and extend the catalytic life of a catalyst bed employed in a hydroconversion reaction zone during hydroprocessing. The present invention more particularly further provides for a method for presulfiding hydroprocessing catalyst ex-situ with a presulfiding agent comprising H₂S at a temperature in the range of 175-240°C, before transferring presulfided hydroprocessing catalyst into a hydroprocessing reactor system. The method is intended to improve the operability and reduce catalyst fouling rate, and to extend the catalytic life of a generally "packed catalyst bed" in the hydroprocessing reactor system that is preferably capable of onstream catalyst replacement. The methods of the present invention may also be advantageously practiced in hydrocarbon reactor systems that utilize an "expanded catalyst bed", such as the ebullated beds as described in U.S. Patent No. 4,571,326 and U.S. Patent No. 4,744,887.

The following three acceptable reactor technologies are currently available to the industry for hydrogen upgrading of "heavy" hydrocarbon liquid streams: (i) fixed bed reactor systems; (ii) ebullated or expanded type reactor systems which are capable of onstream catalyst replacement and are presently known to industry under the trademarks H-Oil_{R} and LC-Fining_{R}; and (iii) the substantially packed-bed type reactor system having an onstream catalyst replacement system, as more particularly described in U.S. Patent No. 5,076,908 to Stangeland et al, having a common assignee with the current inventions and discoveries. A fixed bed reactor system may be defined as a reactor system having one or more reaction zone(s) of stationary catalyst, through which feed streams of liquid hydrocarbon and hydrogen flow downwardly and concurrently with respect to each other. An ebullated or expanded bed system may be defined as a reactor system having an upflow type single reaction zone reactor containing catalyst in random motion in an expanded catalytic bed state, typically expanded from 10% by volume to about 35% or more by volume above a "slumped" bed level which is the volume of a catalytic bed in an ebullated reactor system in a non-expanded or non-ebullated state and without a hydrocarbon stream upflowing therethrough. As particularly described in U. S. Patent No. 5,076,908 to Stangeland et al, the substantially packed-bed type reactor system is an upflow type reactor system including multiple reaction zones of packed catalyst particles having little or no movement during normal use under conditions of no catalyst addition or withdrawal. In the substantially packed-bed type reactor system of Stangeland et al, when catalyst is withdrawn from the reactor during normal catalyst replacement, the catalyst flows in a downwardly direction under essentially plug flow or in an essentially plug flow fashion, with a minimum of mixing with catalyst in layers which are adjacent either above or below the catalyst layer under observation.

It is well know to those skilled in the art of hydrogen upgrading of heavy hydrocarbon liquid streams that catalyst utilized for hydrodemetallation, hydrodesulfurization, hydrodenitrogenation, hydrocracking, etc., of heavy oils and the like are generally made up of a carrier of base material, such as alumina, silica, silica-alumina, or possibly, crystalline aluminosilicate, with one or more promoter(s) or catalytically active metal(s) (or compound(s)) plus trace materials. Typical catalytically active metals utilized are cobalt, molybdenum, nickel and tungsten; however, other metals or compounds could be selected dependent on the application. It is also well know to those skilled in the art of upgrading of heavy oils that potential catalyst activity and useful life can be substantially influenced by the manner in which fresh catalyst is prepared and/or conditioned prior to being exposed to normal reactor operating conditions. More specifically, promoter or catalytically active metals contained in fresh catalyst are in an oxide state. During use for hydroprocessing a sulfur containing feed, the metal oxides are converted to metal sulfides. Catalytic performance of these metal sulfides is generally improved when the oxides in the fresh catalyst are converted to sulfides prior to exposure to reactor operating conditions, using a process termed catalyst presulfiding. Specific procedures have been developed over time by those involved in the industry to presulfide the fresh catalyst charges of fixed bed type reactor systems in-situ at the start of each run. These procedures normally involve a gas heatup and catalyst drying procedure of catalyst in the reactor vessel, followed by catalyst wetting/soaking with startup oil, and then subsequently proceeding to a sulfiding step that employs either non-spiked feedstock (a feedstock containing naturally occurring sulfur compounds) and a sulfur spiked feedstock (a feedstock to which sulfur compounds are added). The sulfiding (or presulfiding) step may also and alternatively employ H₂/H₂S for vapor phase sulfiding. The techniques, as well as several other approaches, are presented and discussed in a technical paper by Harman Hallie at a catalyst symposium in Amsterdam, May 1982, and printed in the December 20, 1982 issue of **Oil and Gas Journal**, and in another paper presented by William J. Tuzynski, at the 1989 NPRA Meeting, and entitled **Properties and Application of Commercial Presulfiding Agents.**

Generally, non-spiked feedstock presulfiding techniques involve decomposition of sulfur compounds, which are naturally present in a selected startup hydrocarbon feed, into H₂S at reactor temperature conditions ranging from about 300°C (572°F) to about 350°C (662°F). Spiked feedstock presulfiding techniques are carried out by injecting sulfur-containing organic compounds into a selected startup hydrocarbon feed such that the injected sulfur-containing organic may decompose into H₂S at temperatures lower than temperatures required to decompose the naturally occurring sulfur compounds present in the startup oil feedstock. Spiking agents currently preferred by the industry are dimethylsulfide (DMS) and dimethyldisulfide (DMDS) which allow sulfiding procedures to be accomplished typically at temperatures in the range of from about 250°C to about 275°C. Vapor phase presulfiding is difficult to control and, in general, does not achieve the optimum results in commercial applications, due to several reasons including poor distribution and uneven sulfiding, poor heat sink of exothermic reactions, etc.

Techniques have been developed in which catalyst is pretreated by impregnation with a sulfur compound (e.g. a polysulfide) before being charged to a reactor for so-called ex-situ presulfiding; however, the catalyst must still undergo drying, wetting, and conversion in-situ from a metal oxide state to a metal sulfide state within the reactor during startup procedures. In this case, the major benefit claimed is reduced startup time and potentially improved activity. U.S. Patent No. 4,576,710 suggests presulfiding regenerated catalyst for use in an ebullating bed reactor, but provides no disclosure of the mechanical details or operating practice to make such a presulfiding step functional.

Conventional presulfiding and startup procedures are tailored to maintain startup oil feed quality and reactor temperature conditions such that the sulfiding and hydrogenation reactions do not create deleterious temperature conditions in the interior of catalyst pellets that result in either carbon deposition or metal sintering, both of which reduce catalyst activity. Simply stated, the severity of hydrogenation reactions during the initial catalyst conditioning and sulfiding period is limited by startup oil quality (e.g. sulfur content) and reactor temperature conditions until the sulfiding reactions diminish or essentially stop. Present-day state-of-the-art techniques allow in-situ presulfiding to be initiated at temperatures below about 200°C (392°F) and completed before temperatures are elevated above about 300°C (572°F). Harman Hallie's technical paper in the December 20, 1982 issue of **Oil and Gas Journal** indicates catalyst activity differences or reductions of from 7% to about 33% could be experience if sulfiding is carried out at higher temperature conditions. Such activity losses may occur when fresh or regenerated catalyst batches with promoter metal in an oxide state are suddenly loaded into an onstream reactor operating at temperatures in excess of 300°C. Therefore, what is needed and what has been invented by us is a viable, reasonably achievable and economical method for presulfiding fresh batches of catalyst which are to be added to an onstream reactor operating at elevated temperatures and hydrogen pressures. A substantial benefit can be gained from preconditioning fresh or regenerated catalyst in order to convert a major portion of the promoter metal oxide into the metal sulfide state prior to its being loaded into an onstream reactor operating at elevated temperatures and hydrogen pressures.

US-A-3 873 441 discloses a process for the catalytic treatment of heavy mineral oils in a moving-bed reactor. Catalyst is sulfided in a lock hopper from which it is conveyed via a second lock hopper to the reaction vessel.

EP-A-785 022 discloses processes for pre-sulfiding hydrocarbon treatment catalysts.

### Summary of the Invention

The present invention provides a method for the extension of cycle length of a catalyst employed in the hydroprocessing of a heavy hydrocarbon feed as defined in claim 1, and to a method for hydroprocessing a heavy hydrocarbon feed as defined in claim 9.

The moving bed reactor comprises at least one reaction zone containing catalytic particulates. Included in the moving bed reactor are means for removing catalytic particulates from the reaction zone and means for adding catalytic particulates to the reaction zone while maintaining the reaction zone at a temperature and at a pressure selected for hydroconverting a refinery stream. During the hydroconversion process, a refinery stream in combination with added hydrogen gas is contacted over catalytic particulates within the reaction zone for removing contaminants from the refinery stream, including one or more of nitrogen, sulfur, aromatics and metals. The effluent from the reaction zone is therefore reduced in one or more of the contaminants relative to the feedstock to the reaction zone.

It is a feature of the moving bed reactor that at least a portion of the catalytic particulates may be removed from the reaction zone during hydroconversion, and further catalytic particulates may be added to the reaction zone during hydroprocessing. Being able to add and remove catalytic particulates without the need for shutting down the reaction process permits the operator to quickly tailor a bed of catalytic particulates for achieving a desired product slate or catalyst activity without the burden of a complete reactor shutdown to replace catalyst. The moving bed reactor also permits the operator to convert refinery streams, such as metals containing streams, which would otherwise quickly deactivate a catalyst. Frequent shutdowns to remove metal fouled catalyst is a major expense for operators of conventional fixed bed hydroconversion processes.

The preferred treatment zone for the catalyst sulfiding system comprises one or more treatment vessels which are separate from the hydroconversion reaction zone contained in the reactor vessel. The preferred pressure is in the range from 200 KPa (15 psig) up to or slightly above (e.g. less than 450 KPa or 50 psig above) the pressure of the reaction zone .

An important aspect of the present invention is the method of preparing and use of a presulfided catalyst in a moving bed reaction system. In conventional fixed bed processes, fresh catalytic particulates are generally sulfided in the reaction vessel prior to the introduction of a refinery stream for reaction. In reaction systems permitting catalyst addition during hydroprocessing, fresh catalysts are conventionally added in an unsulfided state to the reaction zone, and are sulfided by the sulfur compounds present in the fluids flowing through the catalytic particulates during reaction. However, the need for more hydroconversion activity while processing heavy feeds has resulted in the use of catalysts which benefit from careful sulfiding prior to exposure to the heavy feeds at reaction conditions.

In the preferred process of the invention, the method of adding the volume of hydroprocessing catalyst to the treatment zone comprises the steps of:
preparing a slurry comprising a hydrocarbon liquid and a volume of hydroprocessing catalyst;
adding the slurry comprising the hydrocarbon liquid and the hydroprocessing catalyst to the treatment zone; and
removing at least a portion of the hydrocarbon liquid from the treatment zone.
and the method of adding a sulfiding agent to the treatment zone comprises:
pressurizing the treatment zone which contains the hydroprocessing catalyst with a sulfiding agent at a pressure in the range of 0.2 to 24.2 MPa and a temperature in the range of 175°C to 240°C to produce at least partially sulfided catalyst; and
removing at least a portion of the sulfiding agent from the treatment zone.

In a further embodiment of the invention, the process for sulfiding the catalyst in the treatment zone includes flowing a fluid comprising the sulfiding agent through the catalyst within the treatment zone, in a process comprising:
adding a volume of hydroprocessing catalyst to the treatment zone, which volume includes fresh hydroprocessing catalyst;
flowing a heated hydrocarbon liquid through the volume of hydroprocessing catalyst within the treatment zone until the catalyst has a temperature ranging from 90°C to 145°C;
subsequently pressurizing the treatment zone at a pressure ranging from 0.2 MPa to 24.2 MPa (15-3500 psig);
continuing to flow the heated hydrocarbon liquid through the catalyst in the treatment zone until the catalyst has a temperature ranging from 175°C to 240°C;
flowing a sulfiding mixture through the catalyst in the treatment zone to prepare at least partially sulfided catalyst.

The preferred pressure is in the range from 200 KPa (15 psig) up to or slightly above (e.g. less than 450 KPa or 50 psig above) the pressure of the reaction zone.

The presulfided catalyst produced in the process is added to a hydroconversion reaction zone while maintaining the reaction zone at a suitable reaction pressure according to the following:
adding a hydrocarbon liquid to the sulfided catalyst in the treatment zone;
forming a slurry comprising the hydrocarbon liquid and at least a portion of the sulfided catalyst; and
adding the slurry of the hydrocarbon liquid and the sulfided catalyst to the hydroconversion reaction zone while maintaining the reaction zone at the reaction pressure.

In a more preferred embodiment, the present invention is directed to a moving bed reaction zone with a substantially packed bed of catalyst. A method for hydroprocessing a hydrocarbon feed stream that is upflowing through a hydroconversion reaction zone having a substantially packed bed of catalyst comprises the steps of:
introducing a hydrocarbon feed stream into a hydroconversion reaction zone having a substantially packed bed of particulate hydroprocessing catalyst to commence upflowing of said hydrocarbon feed stream through said substantially packed bed of the catalyst at a rate of flow such that said substantially packed bed of hydroprocessing catalyst expands to less than 10% by length beyond a substantially full axial length of said substantially packed bed of hydroprocessing catalyst in a packed bed state, and to recover a reaction effluent therefrom;
withdrawing a first volume of the hydroprocessing catalyst from the hydroconversion reaction zone to commence essentially plug-flowing downwardly said substantially packed bed of hydroprocessing catalyst within said hydroconversion reaction zone;
adding a second volume of a particulate hydroprocessing catalyst to a treatment zone, which second volume includes fresh hydroprocessing catalyst;
sulfiding the second volume of hydroprocessing catalyst within the treatment zone to prepare sulfided catalyst by the procedure of claim 1 or 9; and
adding at least a portion of the sulfided catalyst into the hydroconversion reaction zone to replace the withdrawn first volume of catalyst.

The present invention is directed to presulfiding a hydroprocessing catalyst prior to adding the catalyst to a hydroconversion reaction zone. Processes taught in the art sulfide the hydroprocessing catalyst *in situ*, by adding fresh, unsulfided catalyst to the catalyst bed for sulfiding the catalyst using sulfur-containing reactants which pass through the fresh, unsulfided catalyst. Generally, these prior art sulfiding processes are also run at temperature ranges which are higher than those empolyed in the present process. Among other factors, the present invention is based on the surprising discovery that catalysts which are presulfided according to the present process demonstrate substantially higher performance when used for hydroconversion. The present method provides for sulfiding catalyst, using H₂S present in product streams from the hydroconversion process, at low sulfiding temperatures for preparing a catalyst which has higher performance in catalyzing conversion reactions, particularly desulfurization reactions, of heavy feeds. This discovery is particularly important for operating moving bed reactors, and in particular reactors operating with substantially packed bed upflow reactors under plug flow conditions during catalyst addition and withdrawal.

### In the Figures

Fig. 1 illustrates an embodiment of the invention with a high pressure catalyst transfer vessel only for presulfiding the catalyst according to the invention.
Fig. 2 illustrates an embodiment of the invention with a low pressure catalyst transfer vessel and a high pressure catalyst transfer vessel for presulfiding the catalyst according to the invention.
Fig. 3 shows the improved desulfurization performance of a catalyst presulfided according to the invention.

### Detailed Description of the Invention

Referring in detail now to Figs. 1, 2 for preferred embodiments of the present invention, there is seen a catalyst presulfiding system in communication with the catalyst bed **10** of the reactor vessel **11**. The catalyst sulfiding system functions for sulfiding catalyst (i.e. the converting of metallic oxide(s) within the catalyst into metallic sulfide(s)) before the catalyst is introduced into the reactor vessel **11**. In the invention, catalyst is sulfided (i. e. presulfided) in one or more vessels within treatment zone **50**.

The reaction zone **10** contained within reactor vessel **11** is preferably an upflow reaction system, with reacting fluids entering reaction zone **10** through feed inlet **14**, passing upward in upflow mode through reaction zone **10** moving bed reactor, the reaction effluent exiting through conduit **16.** The catalyst presulfiding process is effective for reaction zones operated as a ebullating bed reaction system or as a substantially packed-bed type reactor system having an onstream catalyst replacement system (i.e. having a capability for transferring catalyst to and from the reaction zone at substantially reaction pressure). To maintain the reactor system as a substantially packed-bed type reactor system, the onstream catalyst replacement system is a counterflow processing system where the catalyst and fluid velocity combinations limit bed expansion to less than 10% by length beyond a substantially full axial length of the bed in a packed bed state. It is more preferred that the bed expansion be maintained at less than 5% and more preferred at less than 1% of the substantially full axial length of the bed in a packed bed state. A preferred substantially packed bed type reactor system is taught in U.S. Patent No. 5,076,908.

In the embodiment of the invention depicted in Fig. 1, the catalyst sulfiding system comprises catalyst transfer vessel **304** in communication with catalyst loading hopper **312** for accepting and dispensing hydroprocessing catalyst. Catalyst hopper **312** has a depending conduit **314** communicating therewith and with the high pressure catalyst feed vessel **304** for conducting hydroprocessing catalyst from the catalyst loading hopper **312** to the catalyst feed vessel **304.** The depending conduit **314** is conveniently provided with a valve **318** for regulating catalyst flow therethrough. Catalyst is preferably transferred from catalyst loading hopper **312** to catalyst feed vessel **304** as a slurry in a hydrocarbon oil.

In one embodiment of the invention, the hydroprocessing catalyst to be sulfided within the catalyst transfer vessel **304** is treating with a sulfiding agent comprising H₂S. The "spiking" or sulfiding agent may include suitable spiking or sulfiding agent (e. g. mercaptan compounds, thiophenic compounds, organosulfides, etc.) but is preferably a sulfur rich recycle stream comprising H₂S recovered from the reaction effluent. Sulfur containing materials, such as dimethyldisulfide or dimethylsulfide, may also be used. An example sulfiding agent is a hydrocarbon gas (e. g. methane, ethane, or the like, etc.) that is rich in hydrogen sulfide (H₂S), preferably containing from about 5% by weight to about 80% by weight H₂S. When H₂S is employed as a sulfiding agent in the present process, a preferred H₂S is derived from a recycle stream (not shown) recovered from the reaction effluent **16**. For example, the reaction effluent **16** may be separated into two or more components by boiling point. Further separations may produce a H₂S rich stream, which may be recycled via conduit **328** for use as a sulfiding agent.

As already stated, the catalyst may be transferred from the catalyst hopper **312** to the catalyst transfer vessel **304** in a slurry, where the liquid component of the slurry may be a product stream from the process, such as a flush oil. At least a portion of the oil remaining in the catalyst transfer vessel following transfer of catalyst from the catalyst hopper to the catalyst transfer vessel is preferentially drained from the catalyst transfer vessel prior to introduction of the sulfiding agent, through conduit **310,** in cooperation with valve **311.** In the embodiment shown in Fig. 1, sulfiding agent may be introduced to the catalyst transfer vessel through conduit line **212** in cooperation with valve **213,** or through conduit line **328,** in cooperation with valve 330.

Prior to sulfiding, the catalyst is heated to an elevated temperature of from 175-240°C. The heat may be supplied by the catalyst transfer vessel, heated to an elevated temperature, using an external heating source, such as a steam jacket. Alternatively, the catalyst may be heated prior to addition of catalyst to the transfer vessel, or by using a heated liquid for flowing through the catalyst in the transfer vessel. In the embodiment of Fig. 1, heated hydrocarbon oil may be supplied from flush oil drum, generally illustrated as **356,** through conduit **340,** where the heated oil is supplied to the flush oil drum through conduit **354,** in cooperation with valve **356.**

The "hydrocarbon" (e.g. a gas oil or a flushing oil) for the heated hydrocarbon and the cold hydrocarbon may be any suitable hydrocarbon but is preferably a heavy distillate fraction boiling above 315 °C and more preferably boiling in the range of from 315 °C to 525°C. It will be apparent to one skilled in the art, however, that hydrocarbon oils boiling below that immediately specified will be suitable in the subject preferred embodiment, so long as the oil does not vaporize to any significant extent at sulfiding conditions during the sulfiding process in the high pressure catalyst transfer vessel **304.**

In this preferred embodiment, catalyst transfer vessel **304,** with added catalyst from which at least a portion of the liquid oil used for transporting the catalyst from catalyst hopper **312** is removed, is pressurized with an H₂S containing stream. The H₂S containing stream can be at any pressure from ambient pressure up to the pressure within reactor vessel **11,** such as from 0.2 MPa to 24.2 MPa (15-3500 psig). H₂S contained in a recycle stream will generally have a pressure of from 0.2 MPa to 3.4 MPa (15-500 psig). The sulfiding agent is introduced to the catalyst transfer vessel through either conduit **212** or conduit **328,** and valves associated with conduits leading to the catalyst transfer vessel blocked closed, including valves **307, 311, 323, 318,** and **386.** Valve **213** remains open, and the catalyst transfer vessel is pressurized to the desired pressure, including up to the pressure of the reactor vessel, using hydrogen or a gaseous mixture containing hydrogen, through conduit **212.** At the desired pressure, valve **213** is closed for a time sufficient to sulfide the catalyst in the transfer vessel. During sulfiding the catalyst is maintained at a temperature in the range of 175°C-240°C. Generally, less than 24 hours, preferably less than 10 hours, more preferably less than 5 hours is sufficient to at least partially sulfide the catalyst. The presulfiding process results in sulfiding at least 35% and more preferably at least 50% of the stoichiometric amount of metal oxide sites available on the catalyst.

It may be desirable to further sulfide the catalyst with additional treatments of the sulfiding agent. Additional treatments beyond the first may be performed in essentially the same way as the first treatment. Thus, at the end of the first treatment, the catalyst transfer vessel **304** is depressurized, for example through conduit **212,** and additional sulfiding agent is added to the transfer vessel **304.** As before, the vessel is pressurized with H₂ to the desired pressure, and the catalyst sulfided under pressure for generally less than 24 hours, preferably less than 10 hours, more preferably less than 5 hours. It will be clear to the skilled practitioner that a tradeoff will exist between the concentration of the active sulfur-containing material, such as H₂S, in the sulfiding agent, the pressure employed during sulfiding the time that sulfiding is permitted to take place and the number of sulfiding cycles employed. Greater amounts of sulfiding will be expected at high concentrations of the sulfur containing material, at higher pressures in the sulfiding step, or for processes in which the sulfiding step is conducted for a longer time. The choice of concentration, pressure and time is largely a matter of local conditions; all combinations are to be considered to be within the bounds of the claimed invention, so long as the sulfided catalyst retains a measurable amount of sulfur at the conclusion of the sulfiding process.

Sulfided catalyst which is sulfided in catalyst transfer vessel **304** is generally transported to reactor vessel **10** in a slurry with a hydrocarbon oil. Such oil may be supplied from flush oil drum **356** through conduit **340.** It is desirable that the catalyst be passed to the reactor in a heated state, e.g. 125-325°C, and so heated oil from flush oil drum **356** is generally used. Such oil may be supplied though hot oil supply line **354** in quantities sufficient to immerse at least a portion of the catalyst in oil at a pressure equal to or slightly higher than the pressure in the reactor vessel. Valve **307** is then opened and the catalyst is passed into the reactor vessel at a rate determined by the rate of oil addition via conduit **324** to the catalyst transfer vessel **304.**

In a separate embodiment, catalyst in transfer vessel **304** is sulfided using a sulfiding agent which is flowed through the catalyst in the transfer vessel **304** during the sulfiding process. Either gaseous or liquid sulfiding agents may be used. As before, catalyst loading hopper **312** is provided for accepting and dispensing hydroprocessing catalyst which preferably comprises the catalyst of the present invention. The catalyst loading hopper **312** has a depending conduit **314** communicating therewith and with the high pressure catalyst feed vessel **304** for conducting hydroprocessing catalyst from the catalyst loading hopper **312** to the catalyst feed vessel **304.** The depending conduit **314** is conveniently provided with a valve **318** for regulating catalyst flow therethrough. The high pressure catalyst feed vessel **304** is provided with a high pressure feed conduit **324** with valve **323** for conducting a feed stream into the high pressure catalyst feed vessel **304.**

The high pressure feed conduit **324** communicates with various feed streams that emanate from various conduits. Conduit **328** conducts a "spiking" or sulfiding agent into the high pressure feed conduit **324.** Flow control valve **330** controls the flow of "spiking" or sulfiding agent in the sulfiding system. Conduit **340** conducts a heated hydrocarbon (e.g. a hot gas oil) and is capable of feeding the high pressure feed conduit **324.** Line **340** includes flow control valve **348** for controlling the flow of heated hydrocarbon for admixing as desired in the feed conduit **324** with the spiking" or sulfiding agent originating from conduit **328.** Conduit **350** contains a flow/liquid level control valve **360** and functions for transporting a cold hydrocarbon (e.g. a cold gas oil) to a flush oil drum, generally illustrated as **356.**

Line **362** contains a flow control valve **358** and interconnects the sulfiding system and the conduit **350** for dispensing a cold hydrocarbon from conduit **350** into the sulfiding feed conduit **324** for admixing with the "spiking" or sulfiding agent and the heated hydrocarbon for lowering the overall temperature of a sulfiding agent/heated hydrocarbon mixture, or for flushing or washing through a catalytic bed (not shown) within the high pressure catalyst feed vessel **304** after the catalyst has been presulfided. In a preferred embodiment, the hydroprocessing catalyst is heated by flowing a heated hydrocarbon liquid through the volume of hydroprocessing catalyst within the treatment zone **50** until the catalyst has a temperature ranging from 90°C to 145°C. The treatment zone is subsequently pressurizing at a pressure ranging from 0.2 MPa to 24.2 MPa (15-3500 psig), and heated hydrocarbon liquid is continued to flow through the catalyst in the treatment zone until the catalyst has a temperature ranging from 170°C to 240°C. A sulfiding mixture, delivered via conduit 324 is then flowed through the catalyst in the treatment zone to prepare sulfided catalyst.

The high pressure catalyst feed vessel **304** is formed with a screen **382** in communication with a conduit **384.** Any mixture of heated hydrocarbon and/or cold hydrocarbon and residual (unreacted) "spiking" or sulfiding agent overflowing the high pressure catalyst feed vessel **304** passes through screen **382** and into the conduit **384** for transportation to and dispensing into a flush oil separator **376.** Conduit **384** comprises a flow/pressure control valve **386** for controlling mixture flow through conduit **384** and for controlling operating or working pressures within the high pressure catalyst feed vessel **304.**

The flush oil separator **376** separates any mixture of heated hydrocarbon and/or cold hydrocarbon and residual (unreacted) "spiking" or sulfiding agent into various components. In a preferred embodiment of the invention where the "spiking" or sulfiding agent is an H₂S-rich hydrocarbon gas, the flush oil separator **376** separates mixture(s) of heated hydrocarbon and/or cold hydrocarbon and H₂S-rich hydrocarbon gas into an overhead gas (e.g. methane, ethane, nitrogen, etc. and mixtures thereof), which exits through an exit conduit 396, having flow/pressure control valve **398,** and a recovered liquid hydrocarbon which exits the flush oil separator **376** through an exit conduit **390** that extends from the flush oil separator **376** to conduit **352** where the recovered liquid hydrocarbon is mixed with heated hydrocarbon and/or cold hydrocarbon for introduction into the flush oil drum **356.** A liquid/flow control valve **392** in exit conduit **390** controls the flow of recovered liquid hydrocarbon from the flush oil separator **376** through the exit conduit **390.**

The recovered liquid hydrocarbon from the flush oil separator **376** typically contains residual overhead gas that did not separate out in the flush oil separator **376.** In those typical occurrences, when a mixture of recovered liquid hydrocarbon and heated hydrocarbon and/or cold hydrocarbon is introduced into the flush oil drum **356** from conduit **352,** residual overhead gas separates in the flush oil drum **356** from the mixture and is dispensed through a conduit **414**. Conduit **414** contains a flow/pressure control valve **420** for regulating residual overhead gas flow and for regulating working or operating pressures within the flush oil drum **356**.

In the embodiment of the invention depicted in Fig. 2, the treatment zone for the catalyst sulfiding system comprises two vessels which are separate from the hydroconversion reaction zone contained in the reactor vessel, a low pressure catalyst feed vessel, generally illustrated as **302,** communicating with a high pressure catalyst transfer vessel, generally illustrated as **304,** via a conduit **306** having a valve **308** for controlling the transfer of at least partially sulfided catalyst from the low pressure catalyst feed vessel **302** to the high pressure catalyst transfer vessel **304.** In this embodiment of the invention, the low pressure catalyst feed vessel **302** is provided as an initial vehicle for wetting, preheating, and at least partially presulfiding the hydroprocessing catalyst before the transfer of at least partially presulfided hydroprocessing catalyst from the low pressure catalyst feed vessel **302** through conduit **306** and into the high pressure catalyst transfer vessel **304.** As will be readily apparent from the following description, the high pressure catalyst transfer vessel **304** is provided with sources for continuing to wet, preheat and further sulfide the at least partially presulfided hydroprocessing catalyst, but at higher temperatures and/or pressures which approximate reaction conditions within the reactor vessel **11**. Presulfiding of hydroprocessing catalyst is performed at lower temperatures and pressures than temperatures and pressures required for directly transferring presulfided catalyst into a hydroconversion reaction zone such as that existing within the reactor vessel **11.** Example sulfiding conditions in the low pressure catalyst transfer vessel **302** include a pressure of greater than 200 KPa (15 psig), preferably between 200 KPa and 7000 KPa (15 psig and 1000 psig), and a temperature of 175-240°C. It is to be understood that the scope of the present invention as depicted in Fig. 1 includes disposing fresh (to be sulfided) hydroprocessing catalyst in both the low pressure catalyst feed vessel **302** and the high pressure catalyst transfer vessel **304,** and subsequently sulfiding simultaneously both batches of hydroprocessing catalyst positioned in the two vessels **302** and **304**.

Sulfided catalyst passes from the high pressure catalyst transfer vessel **304** through conduit **305** for deposit into the reactor vessel **11.** The conduit **305** contains a block valve **307.** A catalyst loading hopper **312** is provided for accepting and dispensing hydroprocessing catalyst which preferably comprises the catalyst of the present invention. The catalyst loading hopper **312** has a depending conduit **314** communicating therewith and with the low pressure catalyst feed vessel **302,** or with the high pressure catalyst feed vessel **304** for conducting hydroprocessing catalyst from the catalyst loading hopper **312** to the catalyst feed vessels **302** or **304.** The depending conduit **314** is conveniently provided with a valve **318** for regulating catalyst flow therethrough. The low pressure catalyst feed vessel **302** is provided with a low pressure feed conduit **320** with associated valve **321** for conducting a feed stream into the low pressure catalyst feed vessel **302.** A high pressure feed conduit **324** communicates with the high pressure catalyst transfer vessel **304** for furnishing a feed stream that is to upflow therethrough.

The low pressure feed conduit **320** and the high pressure feed conduit **324** communicate with various feed streams that emanate from various conduits. Conduit **328** conducts a "spiking" or sulfiding agent into the low pressure feed conduit **320** and the high pressure feed conduit **324** via line **329**. Flow control valve **330** controls the flow of "spiking" or sulfiding agent in the sulfiding system. Conduit **340** conducts a heated hydrocarbon (e.g. a hot gas oil) and is capable of feeding the low pressure feed conduit **320** and the high pressure feed conduit **324** through line **329.** Line **340** includes flow control valve **348** for controlling the flow of heated hydrocarbon for admixing as desired in the feed conduits **320** and **324** respectively with the spiking" or sulfiding agent originating from conduit **328.** Conduit **350** contains a flow/liquid level control valve **360** and functions for transporting a cold hydrocarbon (e.g. a cold gas oil) to a flush oil drum, generally illustrated as **356.**

Line **362** contains a flow control valve **358** and interconnects the sulfiding system and the conduit **350** for dispensing a cold hydrocarbon from conduit **350** into the sulfiding feed conduit **329** for admixing with the sulfiding agent and the heated hydrocarbon for lowering the overall temperature of a sulfiding agent/heated hydrocarbon mixture, or for flushing or washing through a catalytic bed (not shown) within the low pressure catalyst feed vessel **302** and/or the high pressure catalyst feed vessel **304** after the catalyst has been presulfided.

Another feature of the invention depicted in Fig. 2 is that fresh (to be sulfided) hydroprocessing catalyst may be dispensed into both the low pressure catalyst feed vessel **302** and the high pressure catalyst transfer vessel **304** and subsequently simultaneously sulfided in the two vessels **302** and **304.** Such positioning of fresh (to be sulfided) hydroprocessing catalyst may be accomplished in any suitable manner such as initially adding a batch of fresh (to be sulfided) hydroprocessing catalyst into the low pressure catalyst feed vessel **302** from the catalyst loading hopper **312** and subsequently transferring via conduit **306** such initially added batch of fresh hydroprocessing catalyst to the high pressure catalyst transfer vessel **304** and refilling the low pressure catalyst feed vessel **302** from the catalyst loading hopper **312** with another batch of fresh (to be sulfided) hydroprocessing catalyst. Alternatively, a second catalyst loading hopper (not shown) may be provided and dedicated to the high pressure catalyst transfer vessel **304** for dispensing fresh (to be sulfided) hydroprocessing catalyst directly into the high pressure catalyst transfer vessel **304** instead of through the low pressure catalyst feed vessel **302.** If two batches of hydroprocessing catalyst are to be sulfided simultaneously in vessels **302** and **304,** flow control valves **330, 348, 358,** and in lines **328, 340, 362,** respectively, are all opened and regulated as necessary and as would be well known to artisans in the art such that mixtures of sulfided agent and heated hydrocarbon and/or cold hydrocarbon are introduced simultaneously into conduits **320** and **324** for simultaneous upflow through fresh (to be sulfided) hydroprocessing catalyst that has been previously positioned in vessels **302** and **304.**

The low pressure catalyst feed vessel **302** is formed with a screen **370** in communication with a conduit **372.** Any mixture of heated hydrocarbon and/or cold hydrocarbon and residual (unreacted) "spiking" or sulfiding agent overflowing the low pressure catalyst feed vessel **302** passes through screen **370** and into the conduit **372** for transportation to and dispensing into a flush oil separator **376.** Conduit **372** comprises a flow/pressure control valve **380** for controlling mixture flow through conduit **372** and for controlling operating or working pressures within the low pressure catalyst feed vessel **302.** The high pressure catalyst transfer vessel **304** is formed with a screen **382** wherethrough any mixture of heated hydrocarbon and/or cold hydrocarbon and residual (unreacted) "spiking" or sulfiding agent may pass and be introduced into a conduit **384** for transportation through conduit **374** to the flush oil separator **376.** The conduit **384** contains a flow/pressure control valve **386** for controlling mixture flow through conduit **384** from the high pressure catalyst transfer vessel **304** and for controlling operating and working pressures within the latter.

The sulfiding process conditions within the low pressure catalyst feed vessel **302** may include an operating pressure ranging from 0.7 KPa to 1480 KPa (0.1-200 psig). The operating temperature is from 175-240°C; more preferably an operating pressure ranging from 200 KPa to 1140 KPa (15-150 psig) is used. Sulfiding process conditions within the high pressure catalyst transfer vessel **304** may include an operating pressure ranging from 0.7 KPa to 24.2 MPa (0.1-3500 psig). The operating temperature is from 175-240°C; more preferably an operating pressure ranging from 7.0 MPa to 24.2 MPa (1000-3500 psig) is used.

In the process, presulfided catalyst from high pressure transfer vessel **304** may be added to the hydroconversion reaction zone through conduit **305.** While not required, it may be desirable to remove a volume of catalyst from the reaction zone **10,** the volume removed being approximately equal to the volume of presulfided catalyst to be added to the reaction zone **10.** The order of operation, whether adding presulfided catalyst followed by removal of at least partially spent catalyst from the reaction zone, or, alternatively, removing at least partially spent catalyst particulates from the reaction zone followed by adding presulfided catalyst to the reaction zone, or, alternatively, removing at least partially spent catalyst particulates from the reaction zone and adding presulfided catalyst particulates to the reaction zone simultaneously, is not critical to the invention, so long as the catalyst volume in the reaction zone does not exceed design capacity. Methods for transferring catalyst to and from a reaction zone which are useful in the present process are disclosed, for example, in U.S. Patent No. 5,498,327.

The at least partially spent catalyst to be withdrawn from the hydroconversion reaction zone **10** is either intermittently or semi-continuously or continuously withdrawn in the hydrocarbon liquid, as defined above, from the reactor vessel **11** and discharged into conduit **198** via valve **94** for transfer to the high pressure catalyst recovery vessel **304.** The withdrawn catalyst will typically be from about 50% to about 95% expended, more preferably from about 70% to about 80% expended, where a 100% presulfided expended catalyst will be fully fouled and will possess essentially no useful hydroconversion activity at reaction conditions in the hydroconversion zone.

The at least partially spent catalyst in the hydrocarbon liquid has a high concentration of catalyst to hydrocarbon liquid, preferably from about 0.2 to about 1.0 pounds (0.09-0.46 kg) of particulate catalyst per pound of catalyst slurry (i.e. weight of withdrawn catalyst plus weight of hydrocarbon liquids), more preferably from about 0.25 to about 0.8 pounds (0.11-0.37 kg) of particulate catalyst per pound of catalyst slurry, most preferably about 0.5 pounds (0.23 kg) of particulate catalyst per pound of catalyst slurry. The hydrocarbon liquids may comprise a liquid hydrocarbon component which has not been converted (into lighter products) or partly converted or a mixture of partly converted and unconverted liquid hydrocarbon components or a mixture of a hydrogen-containing gas component and any of the liquid components.

In the preferred embodiment of a substantially packed catalyst bed, the withdrawn at least partially spent catalyst is a volumetric layer(i. e. the lowermost volumetric layer) of catalyst from the catalyst bed **10** of reactor vessel **11.** As withdrawal commences the particulate catalyst in the catalyst bed **10** plug flows downwardly. As previously indicated, the withdrawn at least partially expended catalyst is transferred in the hydrocarbon liquid (as defined above) to the high pressure catalyst transfer vessel **304** as a concentrated highly dense liquid slurry in laminar flow, in order to avoid undue abrasion of the withdrawn at least partially expended catalyst particles that are being transferred into the catalyst transfer vessel **304** by conduit **198.**

Catalysts useful in the present process are described in detail in U.S. Patent No. 5,472,928. A preferred catalyst comprises an inorganic support which may include zeolites, inorganic oxides, such as silica, alumina, magnesia, titania and mixtures thereof, or any of the amorphous refractory inorganic oxides of Group II, III or IV elements, or compositions of the inorganic oxides. The inorganic support more preferably comprises a porous carrier material, such as alumina, silica, silica-alumina, or crystalline aluminosilicate. Deposited on and/or in the inorganic support or porous carrier material is one or more metals or compounds of metals, such as oxides, where the metals are selected from the groups IB, VB, VIB, VIIB, and VIII of the Periodic System. Typical examples of these metals are iron, cobalt, nickel, tungsten, molybdenum, chromium, vanadium, copper, palladium, and platinum as well as combinations thereof. Preference is given to molybdenum, tungsten, nickel, cobalt, platinum, and palladium and combinations thereof. Suitable examples of catalyst of the preferred type comprise nickel-tungsten, nickel-molybdenum, cobalt-molybdenum or nickel-cobalt-molybdenum deposited on and/or in a porous inorganic oxide selected from the group consisting of silica, alumina, magnesia, zirconia, thoria, boria or hafnia or compositions of the inorganic oxides, such as silica-alumina, silica-magnesia, alumina-magnesia and the like.

The catalyst of the present invention may further comprise additives, such as phosphorus, boron, clays (including pillared clays), boron phosphate or phosphor, and/or halogens, such as fluorine and chlorine. The boron phosphate compound may be present in an amount ranging from about 10 to about 40 percent by weight calculated on the weight of the total catalyst (i.e. inorganic oxide support plus metal oxide(s)), and more preferably ranging from about 15 to about 30 percent by weight, whereas the halogens and phosphor are used in an amount of less than about 10 percent by weight of the total catalyst.

Although the metal components (i.e. cobalt, nickel, molybdenum, etc.) may be present in any suitable amount, the catalyst of the present invention preferably comprises of from about 0.1 to about 60 percent by weight of metal component(s) calculated on the weight of the total catalyst (i.e. inorganic oxide support plus metal oxides) and more preferably of from about 5 to about 50 percent by weight of the total catalyst. The metals of Group VIII are generally applied in a minor quantity ranging from about 0. 1 to about 30 percent by weight, and the metals of Group VIB are generally applied in a major quantity ranging from about 1.25 to about 50 percent by weight. The atomic ratio of the Group VIII and Group VIB metals may vary within wide ranges, preferably from about 0.01 to about 15, more preferably from about 0.05 to about 10, and most preferably from about 0.1 to about 5.

The groups in the Periodic System referred to above are from the Periodic Table of the Elements as published in Lange's Handbook of Chemistry (Twelfth Edition) edited by John A. Dean and copyrighted 1979 by McGraw-Hill, Inc., or as published in The Condensed Chemical Dictionary (Tenth Edition) revised by Gessner G. Hawley and copyrighted 1981 by Litton Educational Publishing Inc.

In a more preferred embodiment for the catalyst, the oxidic hydrotreating catalyst or metal oxide component carried by or borne by the inorganic support or porous carrier material is molybdenum oxide (MoO₃) or a combination of MoO₃ and cobalt oxide (CoO) or a combination of MoO₃ and nickel oxide (NiO) where the MoO₃ is present in the greater amount. The porous inorganic support is more preferably alumina. The MoO₃ is present on the catalyst inorganic support (alumina) in an amount ranging from about 1 to about 60 percent by weight, preferably from about 1 to about 35 percent by weight, more preferably from about 2 to about 8 percent by weight based on the combined weight of the inorganic support and metal oxide(s). When CoO (or NiO) is present it will be in amounts ranging up to about 30 percent by weight, preferably from about 0.5 to about 20 percent by weight, more preferably from about 1 to about 6 percent by weight based on the combined weight of the catalyst inorganic support and metal oxide(s). The oxidic hydrotreating catalyst or metal oxide component may be prepared by depositing aqueous solutions of the metal oxide(s) on the porous inorganic support material and thoroughly drying, or such catalyst may be purchased from various catalyst suppliers. Catalyst preparative techniques in general are conventional and well known and can include impregnation, mulling, co-precipitation and the like, followed by calcination.

In a preferred embodiment of the present invention, the catalyst will have a uniform size which is preferably spherical with a diameter as a mean of a normal Gausian distribution curve ranging from about 1/64 inch (0.4 mm) to about 1/4 inch (6.4 mm), more preferably ranging from about 1/16 inch (1.6 mm) to about 1/8 inch (3.2 mm). To maintain a uniform size particle, it is preferred that at least about 70%, preferably at least about 80%, and more preferably at least about 90% of the catalyst particles be of a size within about 20%, preferably within about 10%, and more preferably within about 5% of the mean catalyst particle size, where the mean particle size is based on the longest dimension of the particle.

From the foregoing discussion it will be clear to the skilled practitioner that, though the catalyst particles of the present process have a uniform size, shape, and density, the chemical and metallurgical nature of the catalyst may change, depending on processing objectives and process conditions selected. For example, a catalyst selected for a demetallation application with minimum hydrocracking desired could be quite different in nature from a catalyst selected if maximum hydrodesulfurization and hydrocracking are the processing objectives. The type of catalyst selected in accordance with and having the properties mentioned above, is disposed in any hydroconversion reaction zone. A hydrocarbon feed stream is passed through the catalyst, preferably passed through such as to upflow through the catalyst, in order to hydroprocess the hydrocarbon feed stream. More preferably, the catalyst is employed with the various embodiments of the present invention.

The process of the present invention is further illustrated with the following specific example of the invention. In the example process, a hydrocarbon feed stream having a boiling point of greater than about 343°C and containing greater than 1 ppm metals and greater than 500 ppm sulfur is introduced into a hydroconversion reaction zone which contains particulate hydroprocessing catalyst maintained at a reaction pressure, to commence upflowing of said hydrocarbon feed stream through said catalyst and to recover a reaction effluent therefrom. The properties of the feed stream, the properties of the catalyst and reaction conditions, including flow rate, reaction temperature and reaction pressure, are selected to maintain the reactor system as a substantially packed-bed type reactor system, where the catalyst and fluid velocity combinations limit bed expansion to less than 10% by length beyond a substantially full axial length of the bed in a packed bed state. It is more preferred that the bed expansion be maintained at less than 5% and more preferred at less than 1% of the substantially full axial length of the bed in a packed bed state. A preferred reaction pressure in the hydroconversion reaction zone is greater than 343°C, and more preferably in the range of 343°C to 482°C. A preferred reaction pressure in the hydroconversion reaction zone is greater than 7.0 MPa (1000 psig), and more preferably in the range of 7.0 MPa to 24.2 MPa (1000-3500 psig).

During the hydroprocess, a volume of hydroprocessing catalyst within a treatment zone is sulfided to produce sulfided catalyst, and at least a portion of the sulfided catalyst is added into the hydroconversion reaction zone while maintaining the reaction zone at the reaction pressure.

The hydroprocessing catalyst to be sulfided is either fresh hydroprocessing catalyst or combinations of fresh hydroprocessing catalyst and regenerated hydroprocessing catalyst. While additional components other than catalyst to be sulfided may be included in the volume of hydroprocessing catalyst, it is generally not preferred. A volume of the hydroprocessing catalyst is added to a treatment zone, such as by adding a slurry comprising a hydrocarbon liquid and the volume of hydroprocessing catalyst to the treatment zone and removing at least a portion of the hydrocarbon liquid from the treatment zone., and the volume is heated until the catalyst has a temperature ranging from 175°C to 240°C. When the desired temperature is achieved, a sulfiding agent comprising H₂S is added to the treatment zone to prepare sulfided catalyst. A suitable sulfiding agent includes H₂S and H₂, typically in a molar ratio in the range 10:1 to 1:10.

An example method of adding sulfiding agent to the treatment zone comprises introducing a H₂S containing gaseous material to the treatment zone, pressurizing the treatment zone which contains the hydroprocessing catalyst with a H₂ containing gas at a pressure in the range of 200 KPa to 20,000 KPa and a temperature in the range of 175°C to 240°C. The catalyst in the treatment zone is maintained at the given pressure in contact with the sulfiding agent for a sufficient time, generally less than 24 hours, preferably less than 10 hours, more preferably less than 5 hours, to at least partially sulfide the catalyst. The pressure in the treatment zone is then reduced and at least a portion of the sulfiding agent is removed from the treatment zone.

An alternative example method of adding sulfiding agent to the treatment zone comprises adding a volume of hydroprocessing catalyst to the treatment zone, which volume includes fresh hydroprocessing catalyst; flowing a heated hydrocarbon liquid through the volume of hydroprocessing catalyst within the treatment zone until the catalyst has a temperature ranging from 90°C to 150°C; subsequently pressurizing the treatment zone at a pressure ranging from 0.2 MPa to 24.2 MPa (15-3500 psig); continuing to flow the heated hydrocarbon liquid through the catalyst in the treatment zone until the catalyst has a temperature ranging from 175°C to 240°C; flowing a sulfiding mixture through the catalyst in the treatment zone to prepare sulfided catalyst.

The sulfided hydroconversion catalyst is added to the hydroconversion reaction zone at a temperature greater than 125°C, preferably greater than 150°C and at a pressure of no less than the reaction pressure of the hydroconversion reaction zone. The method of adding the sulfided hydroconversion catalyst to the hydroconversion reaction zone comprises adding a hydrocarbon liquid to the sulfided catalyst in the treatment zone; forming a slurry comprising the hydrocarbon liquid and at least a portion of the sulfided catalyst; and adding the slurry of the hydrocarbon liquid and the sulfided catalyst to the hydroconversion reaction zone while maintaining the reaction zone at the reaction pressure.

The reaction zone **10** contained within reactor vessel **11** is preferably an upflow reaction system, with reacting fluids entering reaction zone **10** through feed inlet **14,** passing upward in upflow mode through reaction zone **10** moving bed reactor, the reaction effluent exiting through conduit **16.** The catalyst presulfiding process is effective for reaction zones operated as a ebullating bed reaction system or as a substantially packed-bed type reactor system having an onstream catalyst replacement system (i.e. having a capability for transferring catalyst to and from the reaction zone at substantially reaction pressure). To maintain the reactor system as a substantially packed-bed type reactor system, the onstream catalyst replacement system is a counterflow processing system where the catalyst and fluid velocity combinations limit bed expansion to less than 10% by length beyond a substantially full axial length of the bed in a packed bed state. It is more preferred that the bed expansion be maintained at less than 5% and still more preferred at less than 1% of the substantially full axial length of the bed in a packed bed state. A preferred substantially packed bed type reactor system is taught in U.S. Patent No. 5,076,908.

In carrying out the process of a preferred embodiment of the present invention as broadly illustrated in Figs. 1, 2, a minimum average level of catalytic feed upgrading activity for the countercurrently moving catalyst bed (e.g. catalyst bed **10**) as a whole is selected for the particular catalytic upgrading reaction. For a moving bed (e.g. catalyst bed **10**) in a demetallation reaction system, for example, the minimum average upgrading activity level for the catalyst bed is one which removes the necessary amount of metals from the hydrocarbon feed stream when it passes through the moving bed at demetallation conditions. Similarly, for a desulfurization reaction system, the moving catalyst bed (e.g. catalyst bed **10**) removes the necessary amount of sulfur from the hydrocarbon feed stream when it passes through the moving bed at desulfurization conditions. Thus, as will be apparent to those skilled artisans, the minimum average upgrading activity level for a particular reaction system will depend on the desired degree of a contaminant, such as metals, sulfur, nitrogen, asphaltenes, etc., which the refiner desires to remove from the heavy oil feed. The degree of demetallation or desulfurization (or etc.) will typically be set by economics and the downstream processing that the heavy feed will undergo.

A preferred upgrading use of the present invention is for feed demetallation. For such upgrading, the temperatures and pressures within the reaction zone can be those typical for conventional demetallation processing. The pressure is typically above 3.45 MPa (500 psig). The temperature is typically greater than 315°C., and preferably above 371 °C. Generally, the higher the temperature, the faster the metals are removed; but the higher the temperature, the less efficiently the metals capacity of the demetallation catalyst is used. While demetallation reaction can be conducted in the absence of added hydrogen, hydrogen is generally used and therefore requires full and equal distribution into the moving bed along with any gases evolving from the feed. More preferred hydroprocessing conditions within the hydroconversion reaction zone to hydroprocess the hydrocarbon feed stream include a reaction temperature in a temperature range 343°-482°C (650°-900°F) and a reaction pressure in a pressure range of 7.0 MPa to 24.2 MPa (1000-3500 psig).

The invention is illustrated by the following example of a preferred embodiment. A hydrocarbon feed stream in the presence of hydrogen is introduced into a hydroconversion reaction zone which contains particulate hydroprocessing catalyst maintained at a reaction pressure, to commence upflowing of said hydrocarbon feed stream through said catalyst and to recover a reaction effluent therefrom. The reaction pressure is preselected for the particularly process and reactions desired, and is typically greater than 3.6 MPa (500 psig), preferably in the temperature range of 7.0 MPa to 24.2 MPa (1000-3500 psig). The reaction temperature, which is sufficient to hydroprocess the hydrocarbon feed stream, is in a temperature range of 343°-482°C (650°-900°F). In the process, a first volume of the hydroprocessing catalyst from the hydroconversion reaction zone is withdrawn while maintaining the reaction zone at the reaction pressure. Desirably, the hydroconversion reaction zone contains a substantially packed bed of catalyst, which commences to essentially plug-flow downwardly within the hydroconversion reaction zone when the first volume of hydroprocessing catalyst is withdrawn therefrom.

The preferred process further comprises sulfiding a second volume of hydroprocessing catalyst within a treatment zone to produce sulfided catalyst. In one preferred embodiment of the process, sulfided catalyst is produced by adding a second volume of hydroprocessing catalyst to the treatment zone, which second volume includes fresh hydroprocessing catalyst; heating the second volume of hydroprocessing catalyst until the catalyst has a temperature ranging from 175°C to 240°C; and adding a sulfiding agent comprising H₂S to the treatment zone to prepare sulfided catalyst. If catalyst is added to the treatment zone as a slurry in, e.g. a hydrocarbon stream, it may be desired to remove at least a portion of the hydrocarbon stream prior to sulfiding. Sulfiding agent may be added by flowing the agent, or a liquid stream containing the agent, through the catalyst. Alternatively, sulfiding agent may be added by pressurizing a vessel containing the hydroprocessing catalyst in the treatment zone with the sulfiding agent. A sulfiding procedure involving pressurizing the catalyst in the treatment zone with a sulfiding agent for a time sufficient to sulfide the catalyst may include a step of reducing the pressure in the treatment zone, and repressurizing the catalyst in the treatment zone with a second quantity of sulfiding agent, to further sulfide the catalyst. This cycle may be repeated until the catalyst is adequately sulfided for the use desired.

To heat and/or sulfide the catalyst using flowing liquid streams, one preferred embodiment of the invention includes flowing a heated hydrocarbon liquid through the second volume of hydroprocessing catalyst within the treatment zone until the catalyst has a temperature ranging from 90°C to 145°C; subsequently pressurizing the treatment zone; continuing to flow the heated hydrocarbon liquid through the catalyst in the treatment zone until the catalyst has a temperature ranging from 175°C to 240°C; subsequently adding a sulfiding agent into the heated hydrocarbon liquid to produce a sulfiding mixture; flowing the sulfiding mixture through the catalyst in the treatment zone to prepare sulfided catalyst. The sulfiding agents comprises H₂S, such as the H₂S derived from a recycle stream recovered from the reaction effluent, and optionally dimethylsulfide and dimethyldisulfide. Catalyst is sulfided in the present process at 175-240°C. Catalyst may be sulfided in a low pressure vessel in the treatment zone at a pressure of 200 KPa (15 psig) or higher; in a high pressure vessel in the treatment zone at a pressure in the range of, for example, 7.0 MPa to 24.2 MPa (1000 psig to 3500 psig), or in both.

Sulfided catalyst is added to the hydroconversion reaction zone at a pressure higher than the reaction pressure, in order for the catalyst to flow into the reaction zone. Suitably, the catalyst is added to the reaction zone as a slurry in a hydrocarbon stream by adding a hydrocarbon liquid to the sulfided catalyst in the treatment zone; forming a slurry comprising the hydrocarbon liquid and at least a portion of the sulfided catalyst; and adding the slurry of the hydrocarbon liquid and the sulfided catalyst to the hydroconversion reaction zone.

### Examples

The catalytic particulates comprised an alumina porous carrier material or alumina inorganic support. Deposited on and/or in the alumina porous carrier material was an oxidic hydrotreating catalyst component consisting of NiO and/or MoO₃. The Mo was present on and/or in the alumina porous carrier material in an amount of about 3% by wt., based on the combined weight of the alumina porous carrier material and the oxidic hydrotreating catalyst component(s). The Ni was present on and/or in the alumina porous carrier material in an amount of about 1% by wt., based on the combined weight of the alumina porous carrier material and the oxidic hydrotreating catalyst component(s). The surface area of the catalytic particulates was about 120 sq. meters per gram.
The plurality of catalytic particulates were generally spherical with a mean diameter having a value ranging from about 6 Tyler mesh to about 8 Tyler mesh and an aspect ratio of about 1. The mean crush strength of the catalytic particulates was about 5 lbs (2.3 kg) force. The metals loading capacity of the catalyst or plurality of catalytic particulates was about 0.3 grams of metal per cubic centimeter of catalytic particulate bulk volume.

A sample of the catalyst was loaded into a sulfiding reactor, heated at 205°C, and flooded with medium cycle oil (MCO). After 30 minutes the medium cycle oil was drained, and MCO continued to pump over the catalyst with the drain open for an additional 30 minutes. The flow of MCO was stopped and the excess oil allowed to drain from the catalyst. The catalyst in the sulfiding reactor was then pressurized with 13.2 MPa of 5.0 vol% H₂S in H₂ for 2.5 hours. The sulfiding reactor containing the catalyst was then depressurized to 790 KPa and cooled to 38°C. The catalyst was flushed with heptane to remove the remaining MCO, dried and recovered for analysis. The sulfur content as shown in Run A of Table I is a percent of the amount of sulfur present on a catalyst which was sulfided using dimethyldisulfide in a standard liquid sulfiding procedure at 316°C.

Table I also lists the sulfur content on catalysts sulfided using the procedure of Run A as described (e.g. Run B), using the procedure of Run A but without flooding the catalyst initially with MCO (e.g. Run C), using the procedure of Run A but sulfiding at 316°C (e.g. Run D) or at 149°C (e.g. Run E), or at 204°C for 1.25 hours followed by 316°C for 1.25 hours (e.g. Run F). The results in Table I show that, at the conditions of the experiment, the catalyst was adequately sulfided at 204°C using a single contacting cycle. The extent of sulfiding was higher at 204°C than at either 149°C or at 316°C. Two sulfiding cycles gave slightly better results than one cycle. The best results, in terms of extent of sulfiding of the catalyst, occurred with the sulfiding temperature maintained at 204°C for 1.25 hours followed by 316°C for 1.25 hours (Run F). Runs D and E are comparative.

**Table I**

| Run | A | B | C | D* | E* | F |
|---|---|---|---|---|---|---|
| Catalyst Pretreatment | Wetted with medium cycle oil | Wetted with medium cycle oil | Dry | Wetted with medium cycle oil | Wetted with medium cycle oil | Wetted with medium cycle oil |
| Sulfiding temperature | 204°C | 204°C | 204°C | 316°C | 149°C | 204°C/316°C |
| Number of sulfiding cycles | 1 | 2 | 1 | 1 | 1 | 1 |
| Sulfiding time, each cycle | 2.5 hours | 2.5 hours | 2.5 hours | 2.5 hours | 2.5 hours | 2.5 hours |
| Sulfur content of the sulfided catalyst | 76% | 82% | 77% | 62.5% | 69.1% | 90.5% |

| | | | | | | |
|---|---|---|---|---|---|---|
| * comparative | | | | | | |

Three catalyst samples were tested: an H₂S presulfided catalyst sample prepared as in Run A above (Sample G); a catalyst sample presulfided using a standard dimethyldisulfide liquid presulfiding treatment at 316°C (Sample H); and a catalyst sample which was not presulfided (Sample I). Samples H and I are comparative.

Each catalyst sample was dropped into an Arab Heavy Atmospheric Residuum (4.3% Sulfur, 24.6 ppm nickel, 82.4 ppm vanadium and 11.3 API gravity) heated to 371 °C to simulate dropping catalyst into a moving bed reactor at reaction temperature. The catalyst was removed from the residuum after 24 hours, flushed with solvent, dried, and analyzed for the sulfur content remaining..

| Catalyst Sample | Sulfur content on catalyst, wt% |
|---|---|
| G | 2.83 |
| H | 2.79 |
| I | 2.68 |

These results suggest that the total sulfur content was essentially the same on each of the three catalyst samples.
Following the hot oil treatment, catalyst samples G, H and I were tested for desulfurization activity, using an atmospheric residuum feedstock having the following properties

| | |
|---|---|
| Gravity, °API | 8.9 |
| Sulfur, wt% | 4.51 |
| MCR, wt% | 16.6 |
| V, ppm | 358 |
| Ni, ppm | 70 |
| Asphaltenes, wt% | 13.6 |
| Viscosity @ 100°C, cSt | 285 |

The atmospheric residuum feedstock was contacted with H₂ over each catalyst at 13.9 MPa pressure, a flow rate of 0.75 hr⁻¹, and with a once-through hydrogen flow of 760 liters H₂/kg oil. For the first 250 hours, the reaction temperature was maintained at 378°C. Between 250 hours and 750 hours the reaction temperature was maintained at 402°C.

## Claims

1. A method for the extension of cycle length of a catalyst employed in the hydroprocessing of a heavy hydrocarbon liquid stream, the hydroprocessing occurring in a moving bed reactor system having at least one reaction zone and a treatment zone for presulfiding the catalyst, wherein the heavy hydrocarbon stream is upflowing through the reaction zone, which contains the at least partially presulfided catalyst which has been at least partially presulfided within the treatment zone, and wherein the presulfiding of the catalyst in the treatment zone comprises:
a) adding a volume of hydroprocessing catalyst to the treatment zone, which volume includes fresh hydroprocessing catalyst;
b) partially presulfiding the hydroprocessing catalyst with a presulfiding agent comprising H₂S at a temperature in the range of 175°C to 240°C; and
c) optionally further sulfiding the catalyst with additional treatments of the sulfiding agent.

2. The method of Claim 1, the moving bed reactor system being selected from a group consisting of: (i) ebullated and expanded types of reactor systems which are capable of onstream catalyst replacement; and (ii) a substantially packed-bed type reactor system having an onstream catalyst replacement system.

3. The method of Claim 1, in which the heavy hydrocarbon liquid stream is an atmospheric residuum.

4. The method according to Claim 1, wherein the step of adding a volume of hydroprocessing catalyst to the treatment zone comprises:
a) preparing a slurry comprising a hydrocarbon liquid and a volume of hydroprocessing catalyst;
b) adding the slurry comprising the hydrocarbon liquid and the hydroprocessing catalyst to the treatment zone; and
c) removing at least a portion of the hydrocarbon liquid from the treatment zone.

5. The method according to Claim 1, wherein the treatment zone which contains the hydroprocessing catalyst is pressurized with the presulfiding agent at a pressure in the range of 0.2 to 24.2 MPa, and at least a portion of the presulfiding agent is removed from the treatment zone.

6. The method according to Claim 1, wherein the presulfiding agent comprises a gaseous recycle stream containing H₂ and H₂S.

7. The method of Claim 5, wherein the partially presulfided catalyst is produced at a pressure in the range of 5.0 MPa to 20 MPa.

8. The method according to Claim 1, wherein the step of adding a presulfiding agent to the treatment zone comprises:
a) adding a volume of hydroprocessing catalyst to the treatment zone, which volume includes fresh hydroprocessing catalyst;
b) flowing a heated hydrocarbon liquid through the volume of hydroprocessing catalyst within the treatment zone until the catalyst has a temperature ranging from 90°C to 145°C;
c) subsequently pressurizing the treatment zone at a pressure ranging from 0.2 MPa to 24.2 MPa (15-3500 psig);
d) continuing to flow the heated hydrocarbon liquid through the catalyst in the treatment zone until the catalyst has a temperature ranging from 175°C to 240°C;
e) flowing a presulfiding mixture through the catalyst in the treatment zone to prepare the partially presulfided catalyst.

9. A method for hydroprocessing a heavy hydrocarbon feed stream, which results in improved operability, reduced catalyst fouling rate and extended catalytic life of a catalyst bed, comprises upflowing the feed through a hydroconversion reaction zone, wherein the reaction zone is a moving bed reactor system, the method comprising the steps of:
a) introducing a heavy hydrocarbon feed stream in the presence of hydrogen at a reaction.pressure into a hydroconversion reaction zone which contains particulate hydroprocessing catalyst to commence upflowing of said hydrocarbon feed stream through said catalyst and to recover a reaction effluent therefrom;
b) presulfiding a volume of hydroprocessing catalyst within a treatment zone to produce presulfided catalyst, wherein the presulfiding of the catalyst in the treatment zone comprises:
(1) adding a volume of hydroprocessing catalyst to the treatment zone, which volume includes fresh hydroprocessing catalyst;
(2) partially presulfiding the hydroprocessing catalyst with a presulfiding agent comprising H₂S at a temperature in the range of 175-240°C; and
(3) optionally further sulfiding the catalyst with additional treatments of the sulfiding agent; and
c) adding at least a portion of the sulfided catalyst into the hydroconversion reaction zone while maintaining the reaction zone at the reaction pressure.

10. The method according to Claim 9, wherein the step of adding at least a portion of the presulfided catalyst into the hydroconversion reaction zone comprises:
a) adding a hydrocarbon liquid to the presulfided catalyst in the treatment zone;
b) forming a slurry comprising the hydrocarbon liquid and at least a portion of the presulfided catalyst; and
c) adding the slurry of the hydrocarbon liquid and the presulfided catalyst to the hydroconversion reaction zone while maintaining the reaction zone at the reaction pressure.

11. The method of claim 10, wherein the catalyst is at least partially presulfided at a pressure in the range of 0.2 to 7 MPa.

12. The method of Claim 11 further comprising presulfiding the partially presulfided catalyst at a pressure in the range of 7.0 MPa to 24.2 MPa.

13. The method according to Claim 9, wherein the hydroconversion reaction zone is maintained at a reaction temperature range of 343°C - 482°C and a reaction pressure in a pressure range from 7.0 MPa to 24.2 MPa (1000-3500 psig).

14. The process according to Claim 9, wherein the moving bed reaction system is selected from the group consisting of (i)ebullated and expanded types of reactor systems which are capable of ontream catalyst replacement, (ii) a substantially packed-bed type reactor system having an on-stream catalyst replacement system.

15. A method according to claim 14, further comprising the steps of:
a) introducing a hydrocarbon feed stream into a hydroconversion reaction zone having a substantially packed bed of particulate hydroprocessing catalyst to commence upflowing of said hydrocarbon feed stream through said substantially packed bed of the catalyst at a rate of flow such that said substantially packed bed of hydroprocessing catalyst expands to less than 10% by length beyond a substantially full axial length of said substantially packed bed of hydroprocessing catalyst in a packed bed state, and to recover a reaction effluent therefrom;
b) withdrawing a first volume of the hydroprocessing catalyst from the hydroconversion reaction zone to commence essentially plug-flowing downwardly said substantially packed bed of hydroprocessing catalyst within said hydroconversion reaction zone; and
c) adding a second volume of the presulfided catalyst into the hydroconversion reaction zone to replace the withdrawn first volume of catalyst.

16. The method according to Claim 9, wherein the step of adding a presulfiding agent to the treatment zone comprises:
a) adding a volume of hydroprocessing catalyst to the treatment zone, which volume includes fresh hydroprocessing catalyst;
b) flowing a heated hydrocarbon liquid through the volume of hydroprocessing catalyst within the treatment zone until the catalyst has a temperature ranging from 90°C to 145°C;
c) subsequently pressurizing the treatment zone at a pressure ranging from 0.2 MPa to 24.2 MPa (15-3500 psig);
d) continuing to flow the heated hydrocarbon liquid through the catalyst in the treatment zone until the catalyst has a temperature ranging from 175°C to 240°C;
e) flowing a presulfiding mixture through the catalyst in the treatment zone to prepare the partially sulfided catalyst.

## Patentansprüche

1. Verfahren zur Verlängerung der Zykluslänge eines Katalysators zur Hydrobehandlung eines Flüssigstroms schwerer Kohlenwasserstoffe, wobei die Hydrobehandlung erfolgt in einer Bewegtbett-Reaktoranlage mit mindestens einer Umsetzungszone und einer Behandlungszone für ein Vorsulfidieren des Katalysators, wobei der Strom schwerer Kohlenwasserstoffe von unten nach oben die Umsetzungszone durchströmt, welche mindestens partiell vorsulfidierten Katalysator enthält, der in der Behandlungszone mindestens partiell vorsulfidiert ist, wobei das Vorsulfidieren des Katalysators in der Behandlungszone umfasst
a) Zugeben eines Volumens Hydrobehandlungskatalysators in die Behandlungszone, wobei das Volumen frischen Hydrobehandlungskatalysator enthält;
b) partielles Vorsulfidieren des Hydrobehandlungskatalysators mit einem H₂S enthaltend Vorsulfidierungsmittel bei einer Temperatur im Bereich von 175 bis 240°C; und
c) wahlfrei weiteres Sulfidieren des Katalysators durch weitere Behandlungen mit Sulfidierungsmittel.

2. Verfahren nach Anspruch 1, wobei die Bewegtbett-Reaktoranlage ausgewählt ist aus der Gruppe:
(i) Sprudel- und Expansionsbett-Reaktoranlagen, die einen Onstream-Katalysatoraustausch erlauben; und
(ii) Reaktoranlage mit im Wesentlichen gepacktem Bett, das ein Onstream-Katalysatoraustauschsystem besitzt.

3. Verfahren nach Anspruch 1, wobei der Flüssigstrom schwerer Kohlenwasserstoffe Atmosphären-Residuum ist.

4. Verfahren nach Anspruch 1, wobei der Schritt der Zugabe eines Volumens Hydrobehandlungskatalysator zur Behandlungszone umfasst:
a) Bereiten einer Aufschlämmung von flüssigem Kohlenwasserstoff und einem Volumen Hydrobehandlungskatalysator;
b) Zugabe der Aufschlämmung von flüssigem Kohlenwasserstoff und Hydrobehandlungskatalysator in die Behandlungszone; und
c) Entfernen mindestens eines Teils der flüssigen Kohlenwasserstoffs aus der Behandlungszone.

5. Verfahren nach Anspruch 1, wobei die Behandlungszone, die den Hydrobehandlungskatalysator enthält, mit dem Vorsulfidierungsmittel auf einen Druck von 0,2 bis 24,2 MPa unter Druck gesetzt wird und mindestens ein Teil des Vorsulfidierungsmittels aus der Behandlungszone entfernt wird.

6. Verfahren nach Anspruch 1, wobei das Vorsulfidierungsmittel ein gasförmiger Rezyklierstrom ist, der H₂ und H₂S enthält.

7. Verfahren nach Anspruch 5, wobei der partiell vorsulfidierte Katalysator unter einem Druck von 5,0 bis 20 MPa hergestellt wird.

8. Verfahren nach Anspruch 1, wobei der Schritt des Zusetzens eines Vorsulfidierungsmittels zur Behandlungszone umfasst
a) Zugeben eines Volumens Hydrobehandlungskatalysators zur Behandlungszone, wobei das Volumen frischen Hydrobehandlungskatalysator enthält;
b) Leiten von erwärmtem flüssigen Kohlenwasserstoff durch das Volumen Hydrobehandlungskatalysator in der Behandlungszone, bis der Katalysator eine Temperatur von 90 bis 175°C hat;
c) dann unter Druck setzen der Behandlungszone auf einen Druck von 0,2 bis 24,2 MPa (15-3500 psig);
d) fortwährendes Leiten von erwärmtem flüssigen Kohlenwasserstoff durch den Katalysator in der Behandlungszone, bis der Katalysator eine Temperatur von 175 bis 240°C hat;
e) Leiten eines Vorsulfidierungsgemisches durch den Katalysator in der Behandlungszone und Herstellen des partiell vorsulfidierten Katalysators.

9. Verfahren zur Hydrobehandlung eines Zugabestroms schwerer Kohlenwasserstoffe, welches einen besseren Betrieb bewirkt, die Katalysatorfoulingrate vermindert und eine längeren Katalysezeit des Katalysatorbetts erlaubt, umfassend das Leiten der Beschickung von unten nach oben durch eine HydrokonversionsUmsetzungszone, wobei die Umsetzungszone eine Bewegtbett-Reaktoranlage ist, und das Verfahren die Schritte umfasst
a) Einführen eines Zugabestroms schwerer Kohlenwasserstoffe in Gegenwart von Wasserstoff bei Reaktionsdruck in eine Hydrokonversions-Umsetzungszone, die teilchenförmigen Hydrobehandlungskatalysator enthält zum Starten eines Stroms der Kohlenwasserstoffbeschickung von unten nach oben durch den Katalysator und zur Gewinnung eines Umsetzungs-Abstroms hiervon;
b) Vorsulfidieren eines Volumens Hydrobehandlungskatalysators in einer Behandlungszone und Herstellen von vorsulfidiertem Katalysator, wobei das Vorsulfidieren des Katalysators in der Behandlungszone umfasst:
(1) Zugabe eines Volumens Hydrobehandlungskatalysator in die Behandlungszone, wobei das Volumen frischen Hydrobehandlungskatalysator enthält;
(2) partielles Vorsulfidieren des Hydrobehandlungskatalysators mit einem Vorsulfidierungsmittel , enthaltend H₂S, bei einer Temperatur im Bereich von 175 bis 240°C; und
(3) wahlfrei weiteres Sulfidieren des Katalysators durch weitere Behandlungen mit Sulfidierungsmittel; und
c) Zusetzen mindestens eines Teils sulfidierten Katalysators in die Hydrokonversions-Umsetzungszone und gleichzeitig Halten der Umsetzungszone unter Reaktionsdruck.

10. Verfahren nach Anspruch 9, wobei der Schritt der Zugabe von mindestens einem Teil des vorsulfidierten Katalysators in die Hydrokonversions-Umsetzungszone umfasst
a) Zugabe von flüssigem Kohlenwasserstoff zum vorsulfidierten Katalysator in der Behandlungszone;
b) Herstellen einer Aufschlämmung von der Kohlenwasserstoffflüssigkeit und mindestens einen Teil des vorsulfidierten Katalysators; und
c) Zugeben der Aufschlämmung von Kohlenwasserstoffflüssigkeit und vorsulfidierten Katalysator zur Hydrokonversions-Umsetzungszone und dabei Halten der Umsetzungszone bei Reaktionsdruck.

11. Verfahren nach Anspruch 10, wobei der Katalysator mindestens bei einem Druck im Bereich von 0,2 bis 7 MPa teilweise vorsulfidiert ist.

12. Verfahren nach Anspruch 11, zudem umfassend das Vorsulfidieren des teilweise vorsulfidierten Katalysators unter einem Druck im Bereich von 7,0 bis 24,2 MPa.

13. Verfahren nach Anspruch 9, wobei die Hydrokonversions-Reaktionszone bei einer Reaktionstemperatur im Bereich von 343 bis 482°C gehalten wird und unter einem Reaktionsdruck im Bereich von 7,0 MPa bis 24,2 MPa (1000 bis 3500 psig).

14. Verfahren nach Anspruch 9, wobei die Bewegtbett-Reaktoranlage ausgewählt ist aus der Gruppe (i) Sprudelbett- und Expansionsbett-Reaktoranlagen, die einen Onstream-Katalysatoraustausch erlauben, und (ii) Reaktoranlage mit im Wesentlichen gepackten Betten, der ein Onstream-Katalysatoraustauschsystem besitzt.

15. Verfahren nach Anspruch 14, zudem umfassend die Schritte
a) Einführen eines Kohlenwasserstoffzufuhrstroms in eine Hydrokonversions-Umsetzungszone mit einem im Wesentlichen gepackten Bett von teilchenförmigen Hydrobehandlungskatalysator und Starten eines Stroms der Kohlenwasserstoffbeschickung von unten nach oben durch das im Wesentlichen gepackte Katalysatorbett mit einer solchen Fließgeschwindigkeit, dass das im Wesentlichen gepackte Hydrobehandlungskatalysatorbett um wenigstens 10 Längenprozent expandiert und zwar jenseits der im Wesentlichen vollen Axiallänge des im Wesentlichen gepackten Hydrobehandlungskatalysatorbetts im gepackten Bettzustand und Gewinnen eines Reaktionsabstroms hiervon;
b) Abziehen eines ersten Volumens Hydrobehandlungskatalysator aus der Hydrokonversions-Umsetzungszone und Beginnen eines im Wesentlichen Stopfstroms von oben nach unten durch das im Wesentlichen gepackte Bett mit Hydrobehandlungskatalysator in der Hydrokonversions-Umsetzungszone; und
c) Zugabe eines zweiten Volumens vorsulfidierten Katalysators in die Hydrokonversions-Umsetzungszone und Ersetzen des abgezogenen ersten Katalysatorvolumens.

16. Verfahren nach Anspruch 9, wobei der Schritt des Zugabe eines Vorsulfidierungsmittels zur Behandlungszone umfasst
a) Zugabe eines Volumens Hydrobehandlungskatalysators in die Behandlungszone, wobei das Volumen frischen Hydrobehandlungskatalysator enthält;
b) Leiten von erwärmtem flüssigen Kohlenwasserstoff durch das Volumen Hydrobehandlungskatalysator in der Behandlungszone bis der Katalysator eine Temperatur im Bereich von 90 bis 145°C hat;
c) dann unter Druck setzen der Behandlungszone auf einen Druck im Bereich von 0,2 bis 24,2MPa (15-3500 psig);
d) fortdauerndes Leiten von erwärmtem flüssigen Kohlenwasserstoff durch den Katalysator in der Behandlungszone, bis der Katalysator eine Temperatur im Bereich von 175 bis 240°C hat;
e) Leiten eines Vorsulfidierungsgemisches durch den Katalysator in der Behandlungszone und Herstellen des partiell sulfidierten Katalysators.

## Revendications

1. Procédé pour étendre la durée de cycle d'un catalyseur utilisé dans l'hydrotraitement d'un courant liquide d'hydrocarbures lourds, l'hydrotraitement s'effectuant dans un système de réacteur à lit mobile comprenant au moins une zone réactionnelle et une zone de traitement pour la présulfuration du catalyseur, dans lequel le courant d'hydrocarbures lourds présente un écoulement ascendant à travers la zone réactionnelle, qui contient le catalyseur au moins partiellement présulfuré qui a été au moins partiellement présulfuré dans la zone de traitement, et dans lequel la présulfuration du catalyseur dans la zone de traitement comprend :
a) l'introduction d'un volume de catalyseur d'hydrotraitement dans la zone de traitement, volume qui comprend du catalyseur d'hydrotraitement frais ;
b) la présulfuration partielle du catalyseur d'hydrotraitement avec un agent de présulfuration comprenant H₂S à une température comprise dans l'intervalle de 175°C à 240°C ; et
c) facultativement, en outre, la sulfuration du catalyseur par des traitements supplémentaires avec l'agent de sulfuration.

2. Procédé suivant la revendication 1, le système de réacteur à lit mobile étant choisi dans le groupe consistant en : (i) des systèmes de réacteurs du type bouillonnant et à expansion qui permettent un remplacement de catalyseur en cours de fonctionnement ; et (ii) un système de réacteur du type à lit substantiellement tassé comprenant un système de remplacement de catalyseur en cours de fonctionnement.

3. Procédé suivant la revendication 1, dans lequel le courant liquide d'hydrocarbures lourds est un résidu atmosphérique.

4. Procédé suivant la revendication 1, dans lequel l'étape d'introduction d'un volume de catalyseur d'hydrotraitement dans la zone de traitement comprend :
a) la préparation d'une suspension comprenant un liquide hydrocarboné et un volume de catalyseur d'hydrotraitement ;
b) l'introduction de la suspension comprenant le liquide hydrocarboné et le catalyseur d'hydrotraitement dans la zone de traitement ; et
c) l'évacuation d'au moins une partie du liquide hydrocarboné de la zone de traitement.

5. Procédé suivant la revendication 1, dans lequel la zone de traitement qui contient le catalyseur d'hydrotraitement est mise sous pression avec l'agent de présulfuration à une pression comprise dans l'intervalle de 0,2 à 24,2 MPa, et au moins une partie de l'agent de présulfuration est évacuée de la zone de traitement.

6. Procédé suivant la revendication 1, dans lequel l'agent de présulfuration comprend un courant gazeux de recyclage contenant H₂ et H₂S.

7. Procédé suivant la revendication 5, dans lequel le catalyseur partiellement présulfuré est produit à une pression comprise dans l'intervalle de 5,0 MPa à 20 MPa.

8. Procédé suivant la revendication 1, dans lequel l'étape d'introduction d'un agent de présulfuration dans la zone de traitement comprend :
a) l'introduction d'un volume de catalyseur d'hydrotraitement dans la zone de traitement, volume qui comprend du catalyseur d'hydrotraitement frais ;
b) l'écoulement d'un liquide hydrocarboné chauffé à travers le volume de catalyseur d'hydrotraitement dans la zone de traitement jusqu'à ce que le catalyseur soit à une température comprise dans l'intervalle de 90°C à 145°C ;
c) ensuite la mise sous pression dans la zone de traitement à une pression comprise dans l'intervalle de 0,2 MPa à 24,2 MPa (15 à 3500 psig) ;
d) le maintien de l'écoulement du liquide hydrocarboné chauffé à travers le catalyseur dans la zone de traitement jusqu'à ce que le catalyseur soit à une température comprise dans l'intervalle de 175°C à 240°C ;
e) l'écoulement d'un mélange présulfuré à travers le catalyseur dans la zone de traitement pour préparer le catalyseur partiellement présulfuré.

9. Procédé pour l'hydrotraitement d'un courant d'hydrocarbures lourds d'alimentation, ayant pour résultat une capacité de fonctionnement améliorée, une vitesse réduite d'encrassement du catalyseur et une durée de vie catalytique étendue d'un lit de catalyseur, comprenant l'écoulement ascendant de la charge d'alimentation à travers une zone de réaction d'hydroconversion, la zone réactionnelle étant un système de réacteur à lit mobile, procédé comprenant les étapes consistant :
a) à introduire un courant d'hydrocarbures lourds d'alimentation en présence d'hydrogène à une pression réactionnelle dans une zone de réaction d'hydroconversion qui contient un catalyseur d'hydrotraitement en particules pour commencer l'écoulement ascendant dudit courant d'hydrocarbures d'alimentation à travers ledit catalyseur et pour recueillir un effluent réactionnel à partir de celui-ci ;
b) à présulfurer un volume de catalyseur d'hydrotraitement dans une zone de traitement pour produire un catalyseur présulfuré, la présulfuration du catalyseur dans la zone de traitement comprenant :
(1) l'introduction d'un volume de catalyseur d'hydrotraitement dans la zone de traitement, volume qui comprend du catalyseur d'hydrotraitement frais ;
(2) la présulfuration partielle du catalyseur d'hydrotraitement avec un agent de présulfuration comprenant H₂S à une température comprise dans l'intervalle de 175°C à 240°C ; et
(3) facultativement, en outre, la sulfuration du catalyseur par des traitements supplémentaires avec l'agent de sulfuration ; et
c) l'introduction d'au moins une partie du catalyseur sulfuré dans la zone de réaction d'hydroconversion tout en maintenant la zone réactionnelle à la pression réactionnelle.

10. Procédé suivant la revendication 9, dans lequel l'étape d'introduction d'au moins une partie du catalyseur présulfuré dans la zone de réaction d'hydroconversion comprend :
a) l'addition d'un liquide hydrocarboné au catalyseur présulfuré dans la zone de traitement ;
b) la formation d'une suspension comprenant le liquide hydrocarboné et au moins une partie du catalyseur présulfuré ; et
c) l'introduction de la suspension du liquide hydrocarboné et du catalyseur présulfuré dans la zone de réaction d'hydroconversion tout en maintenant la zone réactionnelle à la pression réactionnelle.

11. Procédé suivant la revendication 10, dans lequel le catalyseur est au moins partiellement présulfuré à une pression comprise dans l'intervalle de 0,2 à 7 MPa.

12. Procédé suivant la revendication 11, comprenant en outre la présulfuration du catalyseur partiellement présulfuré à une pression comprise dans l'intervalle de 7,0 MPa à 24,2 MPa.

13. Procédé suivant la revendication 9, dans lequel la zone de réaction d'hydroconversion est maintenue à une température réactionnelle comprise dans l'intervalle de 343°C à 482°C et à une pression réactionnelle comprise dans l'intervalle de pressions de 7,0 MPa à 24,2 MPa (1000 à 3500 psig).

14. Procédé suivant la revendication 9, dans lequel le système réactionnel à lit mobile est choisi dans le groupe consistant en (i) des systèmes de réacteurs du type bouillonnant et à expansion qui permettent le remplacement du catalyseur en cours de fonctionnement, (ii) un système de réacteur du type à lit substantiellement tassé comprenant un système de remplacement de catalyseur en cours de fonctionnement.

15. Procédé suivant la revendication 14, comprenant en outre les étapes consistant :
a) à introduire un courant d'hydrocarbures d'alimentation dans une zone de réaction d'hydroconversion comprenant un lit substantiellement tassé de catalyseur d'hydrotraitement en particules pour commencer l'écoulement ascendant dudit courant d'hydrocarbures d'alimentation à travers ledit lit substantiellement tassé de catalyseur à une vitesse d'écoulement telle que le lit substantiellement tassé de catalyseur d'hydrotraitement subisse une expansion à moins de 10 % en longueur au-delà d'une longueur axiale pratiquement maximale dudit lit substantiellement tassé de catalyseur d'hydrotraitement à l'état de lit tassé, et pour recueillir un effluent réactionnel à partir de celui-ci ;
b) à décharger un premier volume du catalyseur d'hydrotraitement de la zone de réaction d'hydroconversion pour commencer un écoulement descendant essentiellement du type écoulement-bouchon dudit lit substantiellement tassé de catalyseur d'hydrotraitement dans ladite zone de réaction d'hydroconversion ; et
c) à introduire un second volume du catalyseur présulfuré dans la zone de réaction d'hydroconversion pour remplacer le premier volume de catalyseur déchargé.

16. Procédé suivant la revendication 9, dans lequel l'étape d'introduction d'un agent de présulfuration dans la zone de traitement comprend :
a) l'introduction d'un volume de catalyseur d'hydrotraitement dans la zone de traitement, volume qui comprend du catalyseur d'hydrotraitement frais ;
b) l'écoulement d'un liquide hydrocarboné chauffé à travers le volume de catalyseur d'hydrotraitement dans la zone de traitement jusqu'à ce que le catalyseur soit à une température comprise dans l'intervalle de 90°C à 145°C ;
c) ensuite la mise sous la pression dans la zone de traitement à une pression comprise dans l'intervalle de 0,2 MPa à 24,2 MPa (15 à 3500 psig) ;
d) le maintien de l'écoulement du liquide hydrocarboné chauffé à travers le catalyseur de la zone de traitement jusqu'à ce que le catalyseur soit à une température comprise dans l'intervalle de 175°C à 240°C ;
e) l'écoulement d'un mélange de présulfuration à travers le catalyseur dans la zone de traitement pour préparer le catalyseur partiellement sulfuré.
